



US011732322B2

(12) **United States Patent**  
**Yang et al.**

(10) **Patent No.:** **US 11,732,322 B2**  
(45) **Date of Patent:** **Aug. 22, 2023**

(54) **COLD ROLLED STEEL SHEET**

(71) Applicant: **Algoma Steel Inc.**, Sault Sainte Marie (CA)

(72) Inventors: **Shuhe Yang**, Sault Sainte Marie (CA); **Sang Hyun Cho**, Sault Sainte Marie (CA)

(73) Assignee: **Algoma Steel Inc.**, Sault Ste. Marie (CA)

(\*) Notice: Subject to any disclaimer, the term of this patent is extended or adjusted under 35 U.S.C. 154(b) by 0 days.

(21) Appl. No.: **17/584,778**

(22) Filed: **Jan. 26, 2022**

(65) **Prior Publication Data**

US 2022/0243297 A1 Aug. 4, 2022

**Related U.S. Application Data**

(60) Provisional application No. 63/143,448, filed on Jan. 29, 2021.

(51) **Int. Cl.**

**C21D 9/46** (2006.01)  
**C21D 8/02** (2006.01)  
**C21D 6/00** (2006.01)  
**C22C 38/50** (2006.01)  
**C22C 38/48** (2006.01)  
**C22C 38/42** (2006.01)  
**C22C 38/06** (2006.01)  
**C22C 38/04** (2006.01)  
**C22C 38/02** (2006.01)  
**C22C 38/00** (2006.01)  
**C22C 38/44** (2006.01)

(52) **U.S. Cl.**

CPC ..... **C21D 9/46** (2013.01); **C21D 6/004** (2013.01); **C21D 6/005** (2013.01); **C21D 6/008** (2013.01); **C21D 8/0205** (2013.01); **C21D 8/0226** (2013.01); **C21D 8/0236** (2013.01); **C22C 38/001** (2013.01); **C22C**

**38/002** (2013.01); **C22C 38/02** (2013.01); **C22C 38/04** (2013.01); **C22C 38/06** (2013.01); **C22C 38/42** (2013.01); **C22C 38/44** (2013.01); **C22C 38/48** (2013.01); **C22C 38/50** (2013.01); **C21D 2211/005** (2013.01); **C21D 2211/009** (2013.01)

(58) **Field of Classification Search**

None

See application file for complete search history.

(56) **References Cited**

**U.S. PATENT DOCUMENTS**

2015/0337408 A1\* 11/2015 Schulz ..... C22C 38/02  
420/110

\* cited by examiner

*Primary Examiner* — Anthony M Liang

(74) *Attorney, Agent, or Firm* — Dinsmore & Shohl LLP;  
Weston R. Gould

(57) **ABSTRACT**

Provided is a steel sheet having: ferrite and pearlite composing 80% or more, in area fraction, of the microstructure; yield strength of 60 ksi or more; elongation of at least 23%; an n-value of at least 0.14; incidental impurities; and, in weight percent:

C: 0.03~0.10  
Si: 0~0.6  
Mn: 0.5~1.5  
Cu: 0~1.0  
Ni: 0~1.0  
Nb: 0~0.06  
Ti: 0~0.1  
Mo: 0~0.5%  
Cr: 0~1.0  
Al: 0~0.06  
N: 0.0001~0.006  
Ca: 0~0.006  
P: 0~0.02  
S: 0~0.005.

**4 Claims, 6 Drawing Sheets**



Fig.1 Nital Etch-Middle microstructure – Full hard Strip(x200)



Fig. 2 Nital Etch - Middle microstructure annealed (x200)



Fig 3: L-orientation YS Capability



Fig 4 : L-orientation TS Capability



Fig 5: L-orientation Elongation Capability



Fig 6: L-orientation n value Capability



Fig 7: L-orientation Yield Strength vs. Gauge

| #  | ID   | Group | Orient | 2.0S | UTS | 2" | N  | C   | Mn    | S   | P     | S     | Cr    | Ni    | Co    | Mo    | Si    | Ca    | Sn    | N     | Fe    | Cr    | Si    | Al    | Ca/Si | Spot |      |      |
|----|------|-------|--------|------|-----|----|----|-----|-------|-----|-------|-------|-------|-------|-------|-------|-------|-------|-------|-------|-------|-------|-------|-------|-------|------|------|------|
| 1  | AC19 | 3.27  | l      | 465  | 532 | 26 | 65 | 0.1 | 0.058 | 0.8 | 0.003 | 0.015 | 0.704 | 0.040 | 0.027 | 0.075 | 0.011 | 0.021 | 0.092 | 0.015 | 0.060 | 0.003 | 0.003 | 0.002 | 1356  | 1221 | 1205 | 0.64 |
| 2  | AC19 | 1.27  | l      | 468  | 540 | 28 | 64 | 0.1 | 0.058 | 0.8 | 0.003 | 0.015 | 0.201 | 0.040 | 0.037 | 0.065 | 0.014 | 0.004 | 0.002 | 0.015 | 0.060 | 0.003 | 0.003 | 0.003 | 1352  | 1215 | 1159 | 0.64 |
| 3  | AC19 | 1.27  | l      | 453  | 532 | 28 | 61 | 0.1 | 0.058 | 0.8 | 0.003 | 0.015 | 0.201 | 0.040 | 0.027 | 0.065 | 0.011 | 0.021 | 0.022 | 0.015 | 0.068 | 0.003 | 0.003 | 0.003 | 1355  | 1211 | 1160 | 0.64 |
| 4  | AC19 | 1.27  | l      | 442  | 511 | 25 | 61 | 0.1 | 0.050 | 0.7 | 0.002 | 0.010 | 0.176 | 0.023 | 0.030 | 0.064 | 0.008 | 0.029 | 0.002 | 0.014 | 0.060 | 0.003 | 0.003 | 0.002 | 1346  | 1217 | 1193 | 0.64 |
| 5  | AC19 | 1.27  | l      | 443  | 515 | 26 | 61 | 0.1 | 0.052 | 0.7 | 0.003 | 0.012 | 0.185 | 0.029 | 0.039 | 0.063 | 0.004 | 0.026 | 0.021 | 0.016 | 0.063 | 0.002 | 0.003 | 0.002 | 1352  | 1218 | 1185 | 0.64 |
| 6  | AC19 | 1.27  | l      | 442  | 509 | 26 | 61 | 0.1 | 0.047 | 0.7 | 0.001 | 0.011 | 0.186 | 0.023 | 0.028 | 0.064 | 0.009 | 0.034 | 0.002 | 0.016 | 0.062 | 0.003 | 0.002 | 0.002 | 1348  | 1216 | 1168 | 0.64 |
| 7  | AC19 | 1.27  | l      | 459  | 532 | 26 | 61 | 0.1 | 0.058 | 0.8 | 0.003 | 0.015 | 0.201 | 0.040 | 0.037 | 0.065 | 0.014 | 0.031 | 0.002 | 0.015 | 0.060 | 0.003 | 0.003 | 0.003 | 1348  | 1215 | 1194 | 0.64 |
| 8  | AC19 | 1.27  | l      | 480  | 539 | 25 | 61 | 0.1 | 0.047 | 0.7 | 0.001 | 0.011 | 0.186 | 0.028 | 0.034 | 0.064 | 0.009 | 0.034 | 0.001 | 0.016 | 0.063 | 0.003 | 0.003 | 0.002 | 1349  | 1219 | 1186 | 0.64 |
| 9  | AC19 | 1.27  | l      | 449  | 520 | 26 | 61 | 0.1 | 0.058 | 0.8 | 0.003 | 0.015 | 0.201 | 0.040 | 0.037 | 0.065 | 0.011 | 0.031 | 0.002 | 0.015 | 0.060 | 0.003 | 0.003 | 0.002 | 1347  | 1219 | 1190 | 0.64 |
| 10 | AC19 | 1.27  | l      | 469  | 530 | 26 | 61 | 0.1 | 0.047 | 0.7 | 0.001 | 0.011 | 0.186 | 0.028 | 0.034 | 0.064 | 0.009 | 0.034 | 0.001 | 0.016 | 0.062 | 0.003 | 0.003 | 0.002 | 1347  | 1219 | 1186 | 0.64 |
| 11 | AC19 | 1.27  | l      | 475  | 536 | 25 | 55 | 0.1 | 0.047 | 0.7 | 0.001 | 0.011 | 0.186 | 0.028 | 0.034 | 0.064 | 0.008 | 0.034 | 0.001 | 0.016 | 0.062 | 0.003 | 0.003 | 0.002 | 1347  | 1219 | 1186 | 0.64 |
| 12 | AC19 | 1.42  | l      | 471  | 530 | 26 | 61 | 0.1 | 0.051 | 0.7 | 0.002 | 0.006 | 0.184 | 0.027 | 0.035 | 0.065 | 0.007 | 0.033 | 0.001 | 0.017 | 0.060 | 0.003 | 0.003 | 0.002 | 1348  | 1219 | 1179 | 0.64 |
| 13 | AC19 | 1.27  | l      | 439  | 532 | 25 | 61 | 0.1 | 0.051 | 0.7 | 0.002 | 0.009 | 0.212 | 0.021 | 0.018 | 0.064 | 0.007 | 0.025 | 0.002 | 0.016 | 0.065 | 0.003 | 0.003 | 0.002 | 1345  | 1209 | 1165 | 0.64 |
| 14 | AC19 | 1.27  | l      | 441  | 518 | 26 | 55 | 0.1 | 0.051 | 0.7 | 0.002 | 0.009 | 0.212 | 0.021 | 0.018 | 0.064 | 0.007 | 0.027 | 0.002 | 0.016 | 0.064 | 0.003 | 0.003 | 0.002 | 1348  | 1205 | 1170 | 0.64 |
| 15 | AC19 | 1.42  | l      | 434  | 505 | 25 | 61 | 0.1 | 0.051 | 0.7 | 0.002 | 0.006 | 0.184 | 0.027 | 0.025 | 0.065 | 0.007 | 0.033 | 0.002 | 0.017 | 0.060 | 0.003 | 0.003 | 0.002 | 1348  | 1214 | 1200 | 0.64 |
| 16 | AC19 | 1.27  | l      | 465  | 520 | 26 | 61 | 0.1 | 0.051 | 0.7 | 0.002 | 0.009 | 0.217 | 0.021 | 0.018 | 0.064 | 0.007 | 0.025 | 0.002 | 0.016 | 0.065 | 0.003 | 0.003 | 0.002 | 1345  | 1211 | 1165 | 0.64 |
| 17 | AC19 | 1.27  | l      | 483  | 544 | 24 | 61 | 0.1 | 0.052 | 0.7 | 0.003 | 0.012 | 0.185 | 0.038 | 0.039 | 0.063 | 0.009 | 0.034 | 0.001 | 0.016 | 0.065 | 0.003 | 0.003 | 0.002 | 1348  | 1209 | 1174 | 0.64 |
| 18 | AC19 | 1.27  | l      | 462  | 529 | 25 | 59 | 0.1 | 0.050 | 0.7 | 0.002 | 0.010 | 0.178 | 0.023 | 0.020 | 0.064 | 0.008 | 0.028 | 0.002 | 0.016 | 0.062 | 0.003 | 0.003 | 0.002 | 1347  | 1215 | 1178 | 0.64 |
| 19 | AC19 | 1.27  | l      | 446  | 514 | 26 | 60 | 0.1 | 0.051 | 0.7 | 0.002 | 0.006 | 0.184 | 0.027 | 0.025 | 0.065 | 0.007 | 0.037 | 0.003 | 0.017 | 0.060 | 0.003 | 0.003 | 0.002 | 1347  | 1214 | 1176 | 0.64 |
| 20 | AC19 | 1.27  | l      | 460  | 526 | 26 | 61 | 0.1 | 0.051 | 0.7 | 0.002 | 0.010 | 0.176 | 0.023 | 0.020 | 0.064 | 0.008 | 0.028 | 0.002 | 0.016 | 0.060 | 0.003 | 0.003 | 0.002 | 1348  | 1213 | 1160 | 0.64 |
| 21 | AC19 | 1.27  | l      | 470  | 537 | 25 | 59 | 0.1 | 0.050 | 0.7 | 0.002 | 0.010 | 0.178 | 0.033 | 0.020 | 0.064 | 0.008 | 0.039 | 0.001 | 0.017 | 0.060 | 0.003 | 0.003 | 0.002 | 1348  | 1215 | 1160 | 0.64 |
| 22 | AC19 | 1.42  | l      | 460  | 515 | 26 | 61 | 0.1 | 0.052 | 0.7 | 0.002 | 0.006 | 0.184 | 0.027 | 0.025 | 0.065 | 0.007 | 0.033 | 0.001 | 0.017 | 0.060 | 0.003 | 0.003 | 0.002 | 1348  | 1218 | 1204 | 0.64 |
| 23 | AC19 | 1.42  | l      | 465  | 519 | 26 | 61 | 0.1 | 0.051 | 0.7 | 0.002 | 0.006 | 0.184 | 0.027 | 0.025 | 0.065 | 0.007 | 0.033 | 0.001 | 0.017 | 0.060 | 0.003 | 0.003 | 0.002 | 1348  | 1217 | 1179 | 0.64 |
| 24 | AC19 | 1.27  | l      | 488  | 532 | 24 | 61 | 0.1 | 0.052 | 0.7 | 0.003 | 0.012 | 0.185 | 0.058 | 0.039 | 0.063 | 0.016 | 0.034 | 0.001 | 0.017 | 0.060 | 0.003 | 0.003 | 0.002 | 1347  | 1214 | 1160 | 0.64 |
| 25 | AC19 | 1.27  | l      | 453  | 522 | 25 | 61 | 0.1 | 0.050 | 0.7 | 0.002 | 0.010 | 0.176 | 0.023 | 0.020 | 0.064 | 0.008 | 0.029 | 0.002 | 0.016 | 0.060 | 0.003 | 0.003 | 0.002 | 1346  | 1217 | 1162 | 0.64 |
| 26 | AC19 | 1.27  | l      | 483  | 552 | 23 | 56 | 0.1 | 0.047 | 0.7 | 0.001 | 0.010 | 0.186 | 0.028 | 0.024 | 0.064 | 0.007 | 0.026 | 0.001 | 0.016 | 0.062 | 0.003 | 0.003 | 0.002 | 1348  | 1218 | 1160 | 0.64 |
| 27 | AC19 | 1.27  | l      | 475  | 544 | 24 | 48 | 0.1 | 0.047 | 0.7 | 0.001 | 0.011 | 0.186 | 0.028 | 0.024 | 0.064 | 0.008 | 0.024 | 0.002 | 0.016 | 0.062 | 0.003 | 0.003 | 0.002 | 1348  | 1216 | 1169 | 0.64 |

०८

|    |      |      |   |     |     |    |     |       |     |       |       |       |       |       |       |       |       |       |       |        |       |        |       |      |      |      |      |
|----|------|------|---|-----|-----|----|-----|-------|-----|-------|-------|-------|-------|-------|-------|-------|-------|-------|-------|--------|-------|--------|-------|------|------|------|------|
| 28 | AC19 | 1.27 | 1 | 467 | 532 | 25 | 0.1 | 0.052 | 0.7 | 0.005 | 0.012 | 0.185 | 0.059 | 0.019 | 0.033 | 0.005 | 0.034 | 0.002 | 0.061 | 0.003  | 0.002 | 0.0303 | 1.650 | 1445 | 1238 | 1462 | 0.64 |
| 29 | AC19 | 1.27 | 1 | 454 | 518 | 25 | 0.1 | 0.050 | 0.7 | 0.007 | 0.010 | 0.178 | 0.053 | 0.020 | 0.034 | 0.008 | 0.029 | 0.002 | 0.059 | 0.003  | 0.002 | 0.0304 | 1.647 | 1446 | 1237 | 1460 | 0.64 |
| 30 | AC19 | 1.42 | 1 | 467 | 523 | 26 | 0.1 | 0.051 | 0.7 | 0.002 | 0.006 | 0.158 | 0.027 | 0.025 | 0.035 | 0.007 | 0.023 | 0.002 | 0.059 | 0.003  | 0.002 | 0.0304 | 1.648 | 1441 | 1222 | 1194 | 0.64 |
| 31 | AC19 | 1.42 | 1 | 430 | 498 | 27 | 0.1 | 0.054 | 0.7 | 0.002 | 0.006 | 0.184 | 0.027 | 0.025 | 0.035 | 0.007 | 0.023 | 0.002 | 0.059 | 0.003  | 0.002 | 0.0304 | 1.648 | 1396 | 1236 | 1192 | 0.64 |
| 32 | AC19 | 1.27 | 1 | 435 | 505 | 27 | 0.1 | 0.052 | 0.7 | 0.003 | 0.012 | 0.165 | 0.039 | 0.019 | 0.034 | 0.009 | 0.034 | 0.002 | 0.061 | 0.003  | 0.002 | 0.0303 | 1.647 | 1446 | 1230 | 1160 | 0.64 |
| 33 | AC19 | 1.27 | 1 | 478 | 536 | 24 | 0.1 | 0.052 | 0.7 | 0.005 | 0.012 | 0.186 | 0.039 | 0.018 | 0.033 | 0.009 | 0.034 | 0.002 | 0.061 | 0.003  | 0.002 | 0.0303 | 1.648 | 1446 | 1235 | 1160 | 0.64 |
| 34 | AC19 | 1.27 | 1 | 487 | 564 | 23 | 0.1 | 0.052 | 0.7 | 0.005 | 0.012 | 0.185 | 0.039 | 0.018 | 0.033 | 0.009 | 0.034 | 0.002 | 0.061 | 0.003  | 0.002 | 0.0303 | 1.648 | 1441 | 1238 | 1187 | 0.64 |
| 35 | AC19 | 1.27 | 1 | 460 | 519 | 26 | 0.1 | 0.052 | 0.7 | 0.003 | 0.012 | 0.186 | 0.039 | 0.019 | 0.033 | 0.009 | 0.034 | 0.002 | 0.061 | 0.003  | 0.002 | 0.0303 | 1.648 | 1396 | 1231 | 1180 | 0.64 |
| 36 | AC19 | 1.27 | 1 | 487 | 546 | 23 | 0.1 | 0.047 | 0.7 | 0.001 | 0.001 | 0.186 | 0.028 | 0.024 | 0.04  | 0.009 | 0.034 | 0.002 | 0.062 | 0.003  | 0.002 | 0.0303 | 1.647 | 1396 | 1204 | 1175 | 0.64 |
| 37 | AC19 | 1.27 | 1 | 448 | 512 | 25 | 0.1 | 0.051 | 0.7 | 0.002 | 0.009 | 0.212 | 0.031 | 0.018 | 0.04  | 0.007 | 0.025 | 0.002 | 0.057 | 0.004  | 0.002 | 0.0303 | 1.648 | 1346 | 1209 | 1153 | 0.64 |
| 38 | AC19 | 1.27 | 1 | 450 | 515 | 24 | 0.1 | 0.047 | 0.7 | 0.001 | 0.011 | 0.186 | 0.028 | 0.024 | 0.04  | 0.009 | 0.034 | 0.002 | 0.062 | 0.016  | 0.002 | 0.0303 | 1.647 | 1348 | 1210 | 1180 | 0.64 |
| 39 | AC19 | 1.27 | 1 | 435 | 509 | 25 | 0.1 | 0.051 | 0.7 | 0.002 | 0.009 | 0.212 | 0.031 | 0.018 | 0.04  | 0.007 | 0.025 | 0.002 | 0.057 | 0.004  | 0.002 | 0.0303 | 1.648 | 1350 | 1205 | 1160 | 0.64 |
| 40 | AC19 | 1.27 | 1 | 471 | 528 | 25 | 0.1 | 0.052 | 0.7 | 0.003 | 0.012 | 0.185 | 0.039 | 0.019 | 0.034 | 0.009 | 0.034 | 0.002 | 0.061 | 0.003  | 0.002 | 0.0303 | 1.647 | 1358 | 1214 | 1189 | 0.64 |
| 41 | AC19 | 1.27 | 1 | 451 | 513 | 25 | 0.1 | 0.051 | 0.7 | 0.002 | 0.008 | 0.212 | 0.031 | 0.018 | 0.04  | 0.010 | 0.025 | 0.002 | 0.057 | 0.004  | 0.002 | 0.0303 | 1.647 | 1348 | 1210 | 1180 | 0.64 |
| 42 | AC19 | 1.27 | 1 | 442 | 499 | 26 | 0.1 | 0.051 | 0.7 | 0.002 | 0.009 | 0.212 | 0.031 | 0.018 | 0.04  | 0.007 | 0.025 | 0.002 | 0.057 | 0.004  | 0.002 | 0.0303 | 1.648 | 1350 | 1205 | 1160 | 0.64 |
| 43 | AC19 | 1.27 | 1 | 509 | 553 | 24 | 0.1 | 0.050 | 0.7 | 0.002 | 0.010 | 0.178 | 0.033 | 0.020 | 0.04  | 0.008 | 0.019 | 0.001 | 0.059 | 0.003  | 0.002 | 0.0303 | 1.647 | 1358 | 1214 | 1189 | 0.64 |
| 44 | AC19 | 1.27 | 1 | 501 | 553 | 24 | 0.1 | 0.050 | 0.7 | 0.002 | 0.010 | 0.178 | 0.033 | 0.020 | 0.04  | 0.008 | 0.029 | 0.002 | 0.059 | 0.003  | 0.002 | 0.0303 | 1.648 | 1355 | 1215 | 1178 | 0.64 |
| 45 | ACN5 | 1.42 | 1 | 509 | 565 | 24 | 0.1 | 0.051 | 0.8 | 0.002 | 0.012 | 0.200 | 0.034 | 0.017 | 0.033 | 0.002 | 0.062 | 0.003 | 0.002 | 0.0303 | 1.647 | 1358   | 1210  | 1177 | 0.64 |      |      |
| 46 | ACN5 | 1.47 | 1 | 458 | 529 | 28 | 0.1 | 0.051 | 0.8 | 0.002 | 0.012 | 0.200 | 0.024 | 0.017 | 0.033 | 0.002 | 0.062 | 0.003 | 0.002 | 0.0303 | 1.647 | 1358   | 1210  | 1177 | 0.64 |      |      |
| 47 | ACN5 | 1.47 | 1 | 469 | 533 | 26 | 0.1 | 0.051 | 0.8 | 0.002 | 0.012 | 0.200 | 0.024 | 0.017 | 0.033 | 0.002 | 0.062 | 0.003 | 0.002 | 0.0303 | 1.647 | 1358   | 1210  | 1177 | 0.64 |      |      |
| 48 | ACN5 | 1.01 | 1 | 474 | 544 | 24 | 0.1 | 0.051 | 0.8 | 0.002 | 0.012 | 0.200 | 0.024 | 0.017 | 0.033 | 0.002 | 0.062 | 0.003 | 0.002 | 0.0303 | 1.647 | 1358   | 1210  | 1177 | 0.64 |      |      |
| 49 | ACN5 | 1.01 | 1 | 458 | 546 | 24 | 0.1 | 0.051 | 0.8 | 0.002 | 0.012 | 0.200 | 0.024 | 0.017 | 0.033 | 0.002 | 0.062 | 0.003 | 0.002 | 0.0303 | 1.647 | 1358   | 1210  | 1177 | 0.64 |      |      |
| 50 | ACN5 | 1.47 | 1 | 480 | 584 | 27 | 0.1 | 0.051 | 0.8 | 0.002 | 0.012 | 0.200 | 0.024 | 0.017 | 0.033 | 0.002 | 0.062 | 0.003 | 0.002 | 0.0303 | 1.648 | 1355   | 1208  | 1181 | 0.70 |      |      |
| 51 | ACN5 | 1.47 | 1 | 498 | 551 | 25 | 0.1 | 0.051 | 0.8 | 0.002 | 0.012 | 0.200 | 0.024 | 0.017 | 0.033 | 0.002 | 0.062 | 0.003 | 0.002 | 0.0303 | 1.648 | 1348   | 1214  | 1183 | 0.70 |      |      |
| 52 | ACN5 | 1.01 | 1 | 473 | 544 | 25 | 0.1 | 0.051 | 0.8 | 0.002 | 0.012 | 0.200 | 0.024 | 0.017 | 0.033 | 0.002 | 0.062 | 0.003 | 0.002 | 0.0303 | 1.645 | 1371   | 1211  | 1160 | 0.70 |      |      |
| 53 | ACN5 | 1.47 | 1 | 468 | 548 | 24 | 0.1 | 0.051 | 0.8 | 0.002 | 0.012 | 0.200 | 0.024 | 0.017 | 0.033 | 0.002 | 0.062 | 0.003 | 0.002 | 0.0303 | 1.647 | 1358   | 1210  | 1177 | 0.64 |      |      |

Fig 8 cont. : Actual Process Parameters

## 1

## COLD ROLLED STEEL SHEET

## CROSS REFERENCE TO RELATED APPLICATIONS

This application depends from and claims priority to U.S. Provisional Application No. 63/143,448 filed Jan. 29, 2021, the entire contents of which are incorporated herein by reference.

## FIELD

The invention relates to cold rolled steel sheet.

## BACKGROUND

Cold rolled steel sheet meeting ASTM A1008 HSLAS-F Gr60 typically has a relatively large amount of Niobium, which is relatively expensive.

## SUMMARY

Forming one aspect of the invention is a cold rolled high strength steel sheet comprising, in weight percent:

|               |             |
|---------------|-------------|
| C: 0.03~0.10  | Al: 0~0.06  |
| Si: 0~0.6     | Ca: 0~0.006 |
| Mn: 0.5~1.5   | P: 0~0.02   |
| Cu: 0~1.0     | S: 0~0.005  |
| Ni: 0~1.0     |             |
| Nb: 0 to 0.06 |             |
| Ti: 0 to 0.1  |             |
| Mo: 0 to 0.5  |             |
| Cr: 0~1.0     |             |

N: 0.0001~0.006

and further comprising iron and incidental impurities, the sheet having: ferrite and pearlite composing 80% or more, in area fraction, of the microstructure; yield strength of 60 ksi or more; elongation of at least 23% and a n-value of at least 0.14.

According to other aspects, the weight percent of Mo is optionally no more than 0.060 and the pearlite content can be 20% or less based on the area fraction.

Forming yet another aspect of the invention is a method for use with a steel slab having, in weight percent:

|               |
|---------------|
| C: 0.03~0.10  |
| Si: 0~0.6     |
| Mn: 0.5~1.5   |
| Cu: 0~1.0     |
| Ni: 0~1.0     |
| Nb: 0 to 0.06 |
| Ti: 0 to 0.1  |
| Mo: 0 to 0.5  |
| Cr: 0~1.0     |
| Al: 0~0.06    |
| Ca: 0~0.006   |
| P: 0~0.02     |
| S: 0~0.005    |

N: 0.0001~0.006

and further comprising iron and incidental impurities, the method comprising:

heating the slab to a temperature of 1050° C. to 1150° C.

to produce a heated slab;

rolling the heated slab once at a rolling reduction rate of 20 to 80% in a temperature range above the austenite recrystallization temperature to produce a rolled slab;

## 2

rolling the rolled slab two or more times at a rolling reduction ratio of 40% to 80% in a temperature range below austenite recrystallization temperature and above Ar3 to produce a rolled sheet;

cooling the rolled sheet at a cooling rate of 20° C. to 50° C./sec to produce a cooled sheet;

hot rolling the cooled sheet at a temperature of 300° C. to 690° C. to produce a hot rolled sheet;

cold-working the hot rolled sheet at a reduction rate of 30% to 80% to produce a cold rolled sheet; and annealing the cold rolled sheet for 10 hours or more at 1300° F. or more.

According to another aspect, the steel slab can have Mo in a weight percent no more than 0.06.

According to another aspect, the austenite grain size in the rolled sheet can be 50 µm or less.

## BRIEF DESCRIPTION OF THE DRAWINGS

FIG. 1: illustrates Nital Etch-Middle microstructure of a sheet material.

FIG. 2: illustrates Nital Etch-Middle microstructure of a sheet material of a finished product according to some aspects as provided herein.

FIG. 3: illustrates L-orientation YS Capability of a sheet material of a finished product according to some aspects as provided herein.

FIG. 4: illustrates L-orientation TS Capability of a sheet material of a finished product according to some aspects as provided herein.

FIG. 5: illustrates L-orientation Elongation Capability of a sheet material of a finished product according to some aspects as provided herein.

FIG. 6: illustrates L-orientation n value Capability of a sheet material of a finished product according to some aspects as provided herein.

FIG. 7: illustrates L-orientation Yield Strength vs. Gauge of a sheet material of a finished product according to some aspects as provided herein.

FIG. 8: illustrates process parameters of a sheet material of a finished product according to some aspects as provided herein.

## DESCRIPTION

Non-limiting embodiments of the invention are hereinafter described.

## Sheet Material

Sheet material according to a non-limiting embodiment of the invention comprises, in weight percent:

|               |             |
|---------------|-------------|
| C: 0.03~0.10  | Ca: 0~0.006 |
| Si: 0~0.6     | P: 0~0.02   |
| Mn: 0.5~1.5   | S: 0~0.005  |
| Cu: 0~1.0     |             |
| Ni: 0~1.0     |             |
| Nb: 0 to 0.06 |             |
| Ti: 0 to 0.1  |             |
| Mo: 0 to 0.06 |             |
| Cr: 0~1.0     |             |
| Al: 0~0.06    |             |

N: 0.0001~0.006

and further comprising iron and incidental impurities, wherein the sheet

has ferrite and pearlite composing 80% or more, in area fraction, of the microstructure

has yield strength of 60 ksi or more  
elongation of at least 23%  
has an n-value of at least 0.14.  
has pearlite content no more than 20% based on area  
fraction.

## Method

The method is for use with a steel slab having, in weight  
percent: C: 0.03~0.10

Si: 0~0.6  
Mn: 0.5~1.5  
Cu: 0~1.0  
Ni: 0~1.0  
Nb: 0 to 0.06  
Ti: 0 to 0.1  
Mo: 0 to 0.06  
Cr: 0~1.0  
Al: 0~0.06  
Ca: 0~0.006  
P: 0~0.02  
S: 0~0.005  
N: 0.0001~0.006

and further comprising iron and incidental impurities, the  
method comprising:

heating the slab to a temperature of 1050° C. to 1150° C.  
to produce a heated slab;  
rolling the heated slab once at a rolling reduction rate of  
20% to 80% in a temperature range above the austenite  
recrystallization temperature to produce a rolled slab;  
rolling the rolled slab two or more times at a rolling  
reduction ratio of 40% to 80% in a temperature range  
below austenite recrystallization temperature and  
above Ar3 to produce a rolled sheet;  
cooling the rolled sheet at a cooling rate of 20° C. to 50°  
C./sec to produce a cooled sheet;  
hot rolling the cooled sheet at a temperature of 300° C. to  
690° C. to produce a hot rolled sheet;  
cold-working the hot rolled sheet at a reduction rate of  
30% to 80% to produce a cold rolled sheet; and  
annealing the cold rolled sheet for 10 hours or more at  
1300° F. or more.

## Experimental

## Liquid metal having the following composition

C: 0.03~0.10  
Si: 0~0.6  
Mn: 0.5 ~1.5  
Cu: 0~1.0  
Ni: 0~1.0  
Nb: 0 to 0.06  
Ti: 0 to 0.1  
Mo: 0 to 0.06%  
Cr: 0~1.0  
Al: 0~0.06  
Ca: 0~0.006  
P: 0~0.02  
S: 0~0.005  
N: 0.0001 ~0.006

and further comprising iron and incidental impurities, was  
cast into 78 millimeter (mm) slab at Algoma Steel, Ontario.  
The slab was cleaned by pickling to remove the oxide layer,  
then used in the following method to produce fifty two (52)  
coils. Briefly, the slab is heated to a temperature of 1050° C.  
to 1150° C. to produce a heated slab; the heated slab is rolled  
once at a rolling reduction rate of 20% to 80% in a  
temperature range above the austenite recrystallization tem-  
perature to produce a rolled slab; the rolled slab is rolled two

or more times at a rolling reduction ratio of 40% to 80% in  
a temperature range below austenite recrystallization tem-  
perature and above Ar3 to produce a rolled sheet; the rolled  
sheet is cooled at a cooling rate of 20° C. to 50° C. / sec to  
produce a cooled sheet; the cooled sheet is hot rolled at a  
temperature of 300° C. to 690° C. to produce a hot rolled  
sheet; the hot rolled sheet is cold-worked at a reduction rate  
of 30% to 80% to produce a cold rolled sheet; and the cold  
rolled sheet is annealed for 10 hours or more at 1300° F. or  
more.

Each coil was tested for coil chemistry, and the process  
parameters were monitored during production; details of the  
same are provided in FIG. 8.

Micros were cut in the longitudinal direction of the rolled  
slab [after cold reduction, preceding annealing] and  
mounted, ground, polished and Nital etched to reveal the  
microstructures, as shown in FIG. 1. The elongated grains  
visible in FIG. 1 clearly demonstrate that large amount of  
permanent deformation induced microstructure of full hard  
strip.

The finished product was also inspected after Nital etching  
as shown in FIG. 2. The fully recovered and recrystallized  
uniaxial grains and partially recovered grains at centerline  
clearly demonstrate that ideal microstructure of post  
annealing.

The fifty two (52) rolls produced were tested for mechani-  
cal properties against SAE J2340 420X; the results are  
provided in FIGS. 3-7. Persons of ordinary skill will appre-  
ciate that, surprisingly, notwithstanding the relatively low  
amounts of Niobium, the coils meet the standard.

Whereas two specific embodiments are herein shown and  
described, persons of ordinary skill will readily appreciate  
that variations are possible. Accordingly, the invention  
should be understood to be limited only by the accompa-  
nying claims, purposively construed.

The invention claimed is:

1. A cold rolled high strength steel sheet comprising, in  
weight percent:  
C: 0.03 to 0.10  
Si: 0 to 0.6  
Mn: 0.5 to 1.5  
Cu: 0 to 1.0  
Ni: 0 to 1.0  
Nb: 0 to 0.06  
Ti: 0 to 0.1  
Mo: 0 to 0.5  
Cr: 0 to 1.0  
Al: 0 to 0.06  
N: 0.0001 to 0.006  
Ca: 0 to 0.006  
P: 0 to 0.02  
S: 0 to 0.005  
and further comprising iron and incidental impurities,  
wherein the sheet has ferrite and pearlite composing 80%

or more, in area fraction, of the microstructure has yield  
strength of 60 ksi or more, elongation of at least 23%,  
and an n-value of at least 0.14.

2. The steel sheet according to claim 1, wherein the  
weight percent of Mo is no more than 0.060.

3. The steel sheet according to claim 1, wherein pearlite  
content is greater than 0% and 20% or less based on the area  
fraction.

4. The steel sheet according to claim 2, wherein pearlite  
content is greater than 0% and 20% or less based on the area  
fraction.